# EUROPEAN PATENT APPLICATION

(11) **EP 3 872 440 A1**
(43) Date of publication of application: **01.09.2021**
(21) Application number: 20275050.1
(22) Date of filing: 27.02.2020
(51) Int. Cl.: F42B 12/80, F42B 33/14, F42B 5/24

(54) **IMPROVEMENTS RELATING TO AMMUNITION**

(71) Applicant: BAE SYSTEMS plc, London SW1Y 5AD (GB)
(72) Inventor: The designation of the inventor has not yet been filed
(74) Representative: BAE SYSTEMS plc Group IP Department

(57) **Abstract**

This invention relates to a improvements relating to munitions, specifically to coating small arms ammunition with decoppering agents, as a replacement in lead free ammunition. There is a method of manufacturing a coated metallic projectile for a rifled barrel, comprising; providing a metallic projectile cup with a coating of a decoppering agent located thereon, to provide a coated metallic projectile cup; causing the coated metallic projectile cup to be drawn through a plurality of dies to form a drawn coated metallic projectile.

## Description

This invention relates to improvements relating to ammunition, specifically to coating small arms ammunition with decoppering agents, as a replacement in lead free ammunition.

When a projectile is fired from a rifled barrel, the projectile must deform as it travels along the barrel, so that material forming part of the projectile is forced into the spaces between the lands that form the rifling. This process is called engraving, and causes a spin to be imparted to the projectile by virtue of the twist of the rifling.

The deformation of the projectile, its travel along the barrel effectively as a force fit to the rifling, the high linear acceleration imparted by the gun propellant on firing, and the consequent high rate of angular acceleration and associated force acting between rifling and projectile all contribute to substantial wear on the barrel. The engraved projectile produces copper, which can cause issues when it deposes on the lands and in the rifling grooves of the barrel.

The use of lead as a decoppering agent is well known. The move to using lead free munitions gives rise to issues of copper, from the projectile jackets, accumulating as deposits in the lands of a rifled barrel. The drive for the absence of lead in rounds, gives rise to a new issue that of a lack of decoppering effect.

According to a first aspect of the invention there is provided a method of manufacturing a decoppering agent coated metallic projectile, for a rifled barrel, comprising
a. providing a metallic projectile cup, coating said cup with a decoppering agent, to provide a coated metallic projectile cup
b. causing the coated metallic projectile cup to be drawn through a plurality of dies to form a drawn coated metallic projectile.

Cups, such as metallic projectile cups, cartridge cups, are well known precursor stock materials, ie engineering components, for the production of projectiles and cartridge cases, used in drawing processes. The metallic projectile cup may be selected from any metal, typically copper or alloys thereof, such as gilding metal.

The method provides a metallic projectile cup with a coating of a decoppering agent located thereon, to provide a coated metallic projectile cup,

The thickness of said decoppering agent on the metallic projectile cup may be in the range of from 0.10 microns to 100microns, more preferably in the range of from 1 micron to 20microns, yet more preferably in the range of from 5 to 15 microns.

The decoppering agent may be selected from any known decoppering agent, such as for example tin, lead, bismuth, in the form of metals, alloys and their compounds, such as oxides, nitrate, subcarbonates, antimonides etc., more preferably tin and tin oxides.

The drawn coated metallic projectile comprises a drawn coated metallic jacket over an inner core. The coated metallic jacket comprises a coating of the decoppering agent, the projectile is formed by drawing the coated metallic projectile cup to form a drawn coated metallic jacket over an inner core.

The inner core may be manufactured from any material such as for example ceramics, alloys, metals. The metals may be such as, for example lead, steel, and tungsten.

The inner core may typically be in the form of a monolithic body, and the material selection will depend partly upon the function that the projectile is to perform.

For example in the case of enhanced performance munition the inner core may be a material with a high Vickers Hardness, such as for example greater than 550 HV, more preferably greater than 570 HV. High Vickers hardness materials may be, such as, metals, ceramics, carbides, and borides. The metals may be selected from hardened steel, tungsten, and their alloys thereof. Carbides may be selected from tungsten carbide. However, there is a move towards lead free rounds, preferably hardened steels may be used.

The drawn outer metallic jacket surrounds the inner core, such as the monolithic body, which defines an outer diameter of said projectile.

The drawn outer jacket, is deformable, and may typically be manufactured from a gilding metal jacket, typically copper or alloys thereof, comprising a coating of decoppering agent located thereon.

The metallic projectile cup has inner and outer walls. The inner walls when formed into the final drawn projectile abut the inner core. The outer walls of the metallic projectile cup form the outer surface of the metallic jacket. The metallic projectile cup, may be coated on the inner wall, outer wall, or entire surfaces.

The drawn outer jacket may start as a coated metallic projectile cup, which may be ductile, and therefore extrudable and may be drawn through a series of dies, and forms around the inner core.

In one arrangement the drawn outer coated metallic jacket may be located over a monolithic body which comprises one or more bands or ridges, such that there are cavities created between the drawn outer coated metallic jacket and the bands or ridges of the monolithic body.

The outer diameter of said coated metallic projectile is substantially equal to an internal diameter of the barrel defined by the lands, and wherein during firing of the projectile the lands of the rifling in the barrel deform the outer coated metallic jacket. Upon firing, deformation of the outer coated metallic jacket is designed to provide the projectile with an interference fit with the rifling lands rifling, so as to provide effective obturation by restricting or preventing the escape of propellant gases past the projectile via the rifling grooves. Regard must also be taken to ensure that the force required to effect the deformation of the jacket material and to propel the projectile along the barrel is not excessive, and therefore the diameter of the inner core, and typically the monolithic body may not be greater than that of the rifling lands.

According to a further aspect of the invention there is provided a method of manufacturing a coated metallic projectile cup, capable of forming a metallic projectile for a rifled barrel, comprising
a. providing a precursor stock material with a coating of a decoppering agent located thereon, to provide a coated precursor stock material,
b. causing the coated precursor stock material to be formed into a coated metallic projectile cup, by rolling, drawing, extrusion, stamping.

The decoppering agent may be applied to the precursor stock material or metallic projectile cup by electrolysis, electroless deposition, vapour deposition, chemical vapour deposition, co-depositing/alloying.

According to a further aspect of the invention there is provided a coated metallic projectile, suitable for a rifled barrel, said projectile comprising an inner core, which comprises an drawn outer coated metallic jacket, wherein said outer coated metallic jacket comprises a drawn coating of a decoppering agent thereon.

The thickness of said decoppering agent on the coated metallic projectile may be in the range of from 0.10 microns to 100microns, more preferably in the range of from 1.0 microns to 20microns, yet more preferably in the range of from 5 to 15 microns.

It is essential that the outer diameter (calibre) of the coated metallic projectile is not increased outside of standard tolerances. The use of the decoppering agent coated projectile cups, ensures that the methodology and process steps are adhered to as for pre-existing manufacturing drawing stations. This ensures that the final outer diameter of the metallic jacket are uniform and uniform with current manufactured (uncoated rounds).

The simple step of coating (uncoated) already formed projectiles with a decoppering agent may require some form of reduction of diameter of the uncoated projectile, to allow for the coating thickness of the decoppering agent. This may lead to changes in the steps of the drawing process. This may lead to requirements of requalification of reduced diameter rounds. The methods disclosed herein overcome and prevent need for requalification.

The use of a metallic projectile cup comprising a coating of decoppering agent, allows the direct formation of a decoppering agent coated metallic projectile. This removes the need of setting up a new process of applying a decoppering agent to a ready formed (uncoated) metallic projectile.

The outer drawn metallic jacket and decoppering agent are both drawn from a decoppering agent coated metallic projectile cup.

The decoppering agent may most conveniently be applied to the projectile, as, this is the part of the round that is exposed to the most heat, friction and interaction with the rifling. However, the cartridge case may also be coated with a decoppering reagent.

According to a further aspect of the invention there is provided a tin coated round, suitable for a rifled barrel, comprising a cartridge case, a copper jacketed projectile, propellant, and ignitor cap, wherein at least one of the cartridge case and/or copper jacketed projectile, comprises a drawn coating of a decoppering agent thereon; preferably both the cartridge case and projectile are both tin coated.

According to a further aspect of the invention there is provided a method of manufacturing a coated metallic cartridge for a rifled barrel, comprising
a. providing a metallic cartridge cup with a coating of a decoppering agent located thereon, to provide a coated metallic cartridge cup,
b. causing the coated metallic cartridge cup to be drawn through a plurality of dies to form a drawn coated metallic cartridge case.

In a specific arrangement, for a 7.62mm projectile. It was found that tin plating thicknesses of 5, 10 and 15micron coated metallic projectile cups did not significantly 'thin out' during the drawing process, along the parallel and boat tail sections of the projectile. There was a modest degree of thinning of the original plating thickness on the ogive section as you move away from the parallel section, but returns to the original plating thickness at the nose.

An arrangement of the invention will now be described by way of example and with reference to the accompanying drawings of which;-
Figure 1 shows a round with a layer of decoppering agent.
Figure 2 shows a method of making the coated metallic projectile cup.
Figure 3 shows a round located in a rifled barrel.
Figure 4 shows a complete round with the projectile of the invention.

As shown in Figure 1, a small arms round 1 comprising an inner core 5, outer jacket 3, an ogival portion 2, and a rearwardly located boat tailed portion 8.

The inner core 5, has a drawn outer jacket 3, the drawn outer jacket 3 comprises a layer of drawn decoppering agent 4, such as tin, on the exterior surface. The total outer diameter 7 defines the calibre, which is the sum of the drawn decoppering agent, drawn outer jacket and inner core.

During the drawing process, a gap 6 is often left between the inner core 5 and the drawn outer jacket 3, the gap 6 may comprise a particulate filler, air gap or ceramics.

As shown in Figure 2, there is provided a precursor stock material 10, such as a sheet of copper 13, with a deposed layer of decoppering agent 14 deposed thereon. Tin plating is a well known process, and the tin may be applied by any known method.

The precursor material 10 may be deformed, punched, pressed to provide a decoppering agent coated metallic projectile cup 20. The cup having a wall 23, with an outer layer of decoppering agent 24, deposed thereon. The cup may then be used directly in a draw process to provide elongated cup 21, which is ready to receive an inner core in opening 22. The walls 23 of the elongate cup, comprise the decoppering agent located on the outer surface of the walls 23.

Alternatively, the decoppering agent deposition may be applied to both surfaces of the precursor stock material. In an alternative arrangement the precursor stock material 10a, comprises a sheet of copper 13, with a deposed layer of decoppering agent 14a. 14b deposed on both sides. The subsequent processing into a metallic projectile cup 20a provides a metallic projectile cup which is enveloped with decoppering agent.

In an alternative arrangement, a ready formed metallic projectile cup 19, may be coated directly with a decoppering agent, either on just the outer surface to provide cup 20 or both the inner and outer surface to provide cup 20a.

As shown in Figure 3, in use the round of ammunition comprising the assembled primed and filled cartridge case 33, together with a projectile 31 are fired from a gun having a rifled barrel 34, in the conventional manner, i.e. by chambering the round within the gun chamber 35, and arranging for the primer cap (not shown) to be struck by a firing pin.

When the projectile passes from the gun chamber into the rifled part of the barrel, by virtue of its greater diameter, the inner core 39 becomes engraved by the rifling 37. The diameter of the monolithic body 39 and associated jacket 32 should preferably be substantially equal to or less than the diameter of the rifling grooves 36, 38 .

The jacket 32 is of a malleable material which can be copper or a copper alloy and comprises a decoppering agent coated thereon. This jacket 32 is of a thickness greater than the depth of the rifling grooves, and is of a relatively softer material than that of the monolithic body 39, it can also engrave more readily, and thus contribute for this reason also to a reduction in the engraving force required. Because the jacket 32 is thicker than the depth of rifling, engraving can take place entirely within the coating so that the hard metal of the monolithic body 39 is kept substantially out of contact with the material forming the rifling of the gun barrel. Therefore, despite the hardness of the material forming the main part of the monolithic body 39, barrel wear from this factor is minimised.

Turning to Fig 4, a round 41 is shown. The cartridge assembly 41 comprises a casing 42 and a decoppering agent coated projectile 44. The casing 42 has a hollow section 46, which will contain propellant for displacement of the projectile 44. The casing 42 further comprises a head 48 at the end opposite to the projectile 44 which comprises a chamber 40 for a percussion cap (not shown), and a flash tube 42 for communication of an ignition charge from the percussion cap to the inside of the casing 42 and thus the propellant. The walls of the chamber 46 are formed integrally with the head 48. The walls 46 of the cartridge case chamber may also be plated with a decoppering agent, on the inner surface, outer surface or both. Such a cartridge casing may typically be formed of brass, steel or titanium.

## Claims

1. A method of manufacturing a decoppering agent coated metallic projectile for a rifled barrel, comprising
a. providing a metallic projectile cup, coating said cup with a decoppering agent, to provide a coated metallic projectile cup,
b. causing the coated metallic projectile cup to be drawn through a plurality of dies to form a drawn coated metallic projectile.

2. A method according to claim 1, wherein the thickness of said decoppering coating on the metallic projectile cup is in the range of from 0.10 microns to 100m icrons.

3. A method according claim 2, wherein the thickness of the coating of a decoppering agent is in the range of from 5 microns to 15 microns.

4. A method according to any one of the preceding claims wherein the decoppering agent is tin.

5. A method according to any one of the preceding claims wherein the drawn coated metallic projectile, comprises an outer jacket, which comprises said decoppering agent, and wherein said outer jacket is drawn over an inner core.

6. A method according to any one of the preceding claims wherein the metallic projectile cup is gilding metal, copper or copper alloys thereof.

7. A method of manufacturing a coated metallic projectile cup, capable of forming a coated metallic projectile for a rifled barrel, comprising
a. providing a precursor stock material with a coating of a decoppering agent located thereon, to provide a coated precursor stock material
b. causing the coated precursor stock material to be formed into a coated metallic projectile cup, by rolling, drawing, extrusion, stamping.

8. A method according to any one of the preceding claims wherein the decoppering agent is applied to the precursor stock material or metallic projectile cup by electrolysis, electroless deposition, vapour deposition, chemical vapour deposition, co-depositing/alloying.

9. A coated metallic projectile, suitable for a rifled barrel, said projectile comprising an outer drawn metallic jacket, said jacket encapsulating an inner core, wherein said outer drawn metallic jacket comprises a drawn coating of a decoppering agent located thereon.

10. A coated metallic projectile according to claim 9, wherein the metallic jacket comprising the decoppering agent located thereon are both drawn from a decoppering agent coated metallic projectile cup, wherein said decoppering agent coating is in thickness in the range of from 0.1 microns to 100microns.

11. A coated metallic projectile according to claim 9 or 10, wherein the thickness of the coating of a decoppering agent is in the range of from 5 microns to 15 microns.

12. A coated metallic projectile according to claim 9 to 11, wherein the drawn projectile metallic jacket is gilding metal, copper, brass, steel, or titanium.

13. A coated metallic projectile cup suitable for use to manufacture a coated metal jacket of a projectile, said metal jacket comprising a coating of a decoppering agent thereon, wherein said coating is in thickness in the range of from 0.10 microns to 100microns.

14. A method of manufacturing a coated metallic cartridge for a rifled barrel, comprising
a. providing a metallic cartridge cup, coating said metallic cartridge with a decoppering agent, to provide a coated metallic cartridge cup,
b. causing the coated metallic cartridge cup to be drawn through a plurality of dies to form a drawn coated metallic cartridge case.

15. A tin coated round, suitable for a rifled barrel, comprising a cartridge case, a copper jacketed projectile, propellant, and ignitor cap, wherein at least one of the cartridge case and/or copper jacketed projectile, comprises a drawn coating of a decoppering agent thereon.
